

P. J. KLOPSCH,  
COMPOSITION BOWLING BALL,  
APPLICATION FILED NOV. 26, 1915.

1,203,747.

Patented Nov. 7, 1916.

*Fig. 1,*



*Fig. 2.*



*Fig. 3.*



WITNESSES

*Edw. Thorpe  
Roy G. Foster*

INVENTOR

*Paul J. Klopsch  
BY *M. M. Co.**

ATTORNEYS

# UNITED STATES PATENT OFFICE.

PAUL J. KLOPSCH, OF BAYONNE, NEW JERSEY.

## COMPOSITION BOWLING-BALL.

1,203,747.

Specification of Letters Patent.

Patented Nov. 7, 1916.

Application filed November 26, 1915. Serial No. 63,454.

*To all whom it may concern:*

Be it known that I, PAUL J. KLOPSCH, a citizen of the United States, and a resident of Bayonne, in the county of Hudson and 5 State of New Jersey, have invented a new and Improved Composition Bowling-Ball, of which the following is a full, clear, and exact description.

The object of the invention is to provide 10 a new and improved composition bowling ball which can be cheaply manufactured, is not liable to wear unduly or chip around the finger holes, and one which is properly balanced, of the correct weight relative to 15 its size, not liable to appreciably shrink or expand under different weather conditions, at the same time having the desired hardness and resiliency.

In order to produce the desired result, 20 use is made of a core and a shell inclosing the core, the latter being formed of chlorid of magnesia and oxid of magnesia in about equal parts, and a filler such as comminuted wood, cork, rope or like material, and the 25 said shell being formed of a condensation product of carbolic acid and formaldehyde such, for instance, as is known in trade under the name of "bakelite," "condensite" and the like.

30 A practical embodiment of the invention is represented in the accompanying drawings forming a part of this specification, in which similar characters of reference indicate corresponding parts in all the views.

35 Figure 1 is a side elevation of the composition bowling ball with parts of the shell shown in section; Fig. 2 is a sectional side elevation of an apparatus illustrating the first step in the manufacture of the bowling 40 ball; and Fig. 3 is a similar view of the same showing the second step in the manufacture of the bowling ball.

The composition bowling ball in its general construction consists of a core 10 and 45 shell 11 tightly inclosing the core 10. The core 10 is formed of a mixture of chlorid of magnesia dissolved in water to a density of about 29° Baumé, oxid of magnesia, and a filler of comminuted wood, sawdust, peat, 50 cork, rope or similar light material. The chlorid of magnesia and the oxid of magnesia are of equal parts and the filler is about 20% in weight, and a pigment likewise of 20% in weight may be added to give 55 a y desired color to the core. Thus when a

black color is desired bone black may be used as a pigment, and for a red color oxid of iron may be used, but I do not limit myself to any one particular pigment. The mixing of the ingredients for the core is 60 carried on under ordinary temperature and the mixture is pressed in a mold to spherical form and then left to dry, so that it becomes very hard in about twenty-four hours. It is understood that the chlorid of magnesia 65 and the oxid of magnesia form about 60% of the weight of the core 10.

The shell 11 is formed of a condensation product of carbolic acid and formaldehyde, such, for instance, as is known in the trade 70 under the name of "bakelite," "condensite" and the like.

In manufacturing the bowling ball use is made of two half molds 12 and 13 having 75 semi-spherical recesses adapted to register with each other to form a spherical recess of the size of the bowling ball to be made. A quantity of the condensation product above mentioned and while in dry powder form is placed in the half mold 12 and then a half-round plunger 14 under a pressure of about 2,000 lbs. is used to press this product in the mold 12 under a heat of about 110° Fahrenheit, into the shape of a half-shell 15, as 80 plainly indicated in Fig. 2. The plunger 14 and the half shell are then removed and a like second half shell 16 is made of the same material and in the same manner. The previously formed core 10 is next inclosed between the half shells 15 and 16 which are 85 now subjected to both pressure and heat in the two half molds 12 and 13, as shown in Fig. 3. Both half molds 12 and 13 are heated to about 350° Fahrenheit, preferably 90 by the use of superheated steam passed into the molds, as indicated in Fig. 3, and at the same time a pressure of about 2,000 lbs. is 95 exerted against the molds to unite the material of the half shells 15 and 16 at the edges thereof and thus form a complete shell 11 tightly around the core 10. It takes but a few minutes to accomplish the shaping and 100 pressing operation in the mold halves 12 and 13, and then the steam is shut off and the molds are allowed to cool, after which they 105 are taken apart to allow removal of the bowling ball, which, after the final cooling, is ready for immediate use. It is evident that under the heavy pressure and the heat the 110 edges of the two half shells completely merge

without leaving any joint whatever and the exterior surface of the shell 11 appears polished. The finished ball may be bored for providing the usual finger holes. It is understood that in practice a number of half shells 15 and 16 can be manufactured in the half mold 12 with the aid of the plunger 14, and a pair of such half shells 15 and 16 can be united around a core 10 in a separate set 10 of molds 12 and 13.

In manufacturing a standard ball of 27 inches in circumference and 16 lbs. in weight, the core 10 is approximately 11 lbs. in weight while the remaining 5 lbs. are supplied by 15 the shell 11, and the latter is about a half inch thick and the core about  $7\frac{1}{16}$  of an inch in diameter. The proportion in weight and size of the core 10 and the shell 11 may, however, be varied especially when forming 20 bowling balls of smaller size.

A bowling ball constructed in the manner described has the requisite properties of a rubber or a boxwood ball, namely, the desired hardness, resiliency, durability and 25 wearing quality.

The bowling ball produced is not liable to chip around the finger holes and is properly balanced and not liable to appreciably shrink or expand under different weather 30 conditions.

A composition bowling ball constructed as set forth can be cheaply manufactured and sold at about one-half the price of an ordinary composition ball as now sold in the 35 market.

Having thus described my invention, I

claim as new and desire to secure by Letters Patent:

1. A composition bowling ball, comprising a core and a shell tightly inclosing the said core, the latter consisting of a cementitious mass and a filler and the shell consisting of a condensation product of carbolic acid and formaldehyde. 40

2. A composition bowling ball, comprising a core and a shell tightly inclosing the said core, the core consisting of a mixture of a solution of chlorid of magnesia, oxid of magnesia and a filler, and the shell consisting of a condensation product of carbolic acid and formaldehyde. 45

3. A composition bowling ball, comprising a core and a shell tightly inclosing the said core, the latter consisting of equal parts of chlorid of magnesia and oxid of magnesia, and a light filling material, and the said shell consisting of a condensation product of carbolic acid and formaldehyde. 55

4. A composition bowling ball, comprising a core and a hard baked shell tightly inclosing the said core, said core consisting of equal parts of chlorid of magnesia and oxid of magnesia and approximately twenty per cent. of a comminuted fibrous filling material. 60

In testimony whereof I have signed my name to this specification in the presence of two subscribing witnesses.

PAUL J. KLOPSCH.

Witnesses:

THEO. G. HOSTER,  
PHILIP D. ROLLHAUS.